

Oct. 8, 1946.

J. J. CROWE

2,409,020

METHOD FOR DESULPHURIZING IRON WITH MOLTEN CALCIUM CARBIDE

Filed Dec. 8, 1943

Fig. 1.



Fig. 2.



INVENTOR.

John J. Crowe

BY

Pennie Davis Marvin & Edwards  
ATTORNEYS

## UNITED STATES PATENT OFFICE

2,409,020

METHOD FOR DESULPHURIZING IRON  
WITH MOLTEN CALCIUM CARBIDEJohn J. Crowe, Westfield, N. J., assignor to Air  
Reduction Company, Incorporated, New York,  
N. Y., a corporation of New York

Application December 8, 1943, Serial No. 513,384

3 Claims. (Cl. 75—58)

1

This invention relates to the desulphurizing of metals such as iron and steel and particularly to an improved method of introducing a desulphurizing agent to molten metal and apparatus therefor.

As is well known, sulphur may be an undesirable element in iron and steel. Various methods of eliminating sulphur have been proposed, including the addition of solid calcium carbide ( $CaC_2$ ) to the molten metal.

The melting point of calcium carbide is approximately  $2300^{\circ} C.$ , which is far above the temperature ordinarily met in a molten metal bath. Moreover, calcium carbide is lighter than iron and when added to a molten metal bath in a solid form, comes to the surface of the bath before dissolving. Hence it is difficult to secure satisfactory diffusion of the added material in the molten metal and combination with the sulphur present.

It is the object of the present invention to provide a simple and effective method of and apparatus for introducing calcium carbide in a molten condition to a bath of molten metal and thereby to facilitate reaction with and reduction of the sulphur content of the metal.

Other objects and advantages of the invention will be apparent as it is better understood by reference to the following specification and the accompanying drawing, in which

Fig. 1 is a vertical sectional view of an apparatus suitable for the practice of the invention; and

Fig. 2 is a section on the line 2—2 of Fig. 1.

I have discovered that calcium carbide can be used successfully as a desulphurizing agent for molten metals, particularly iron, steel and cast iron, by melting the carbide in an electric arc or by the localized resistance to the passage of an electric current in such a manner that the molten carbide is introduced immediately beneath the surface of the molten metal to be treated without exposure to the atmosphere. The agitation produced by the operation of the arc assists in causing the molten carbide to disseminate through the molten metal.

In carrying out the invention, I prefer to employ a melting receptacle for the carbide which floats upon the surface of the molten metal in a ladle or other suitable container. The carbide is melted by heat produced by localized resistance to the passage of an electric current such as an electric arc, and the molten carbide in the bottom of the receptacle is in direct contact with the molten metal. Cooling of the molten carbide

2

by contact with the atmosphere is thus avoided and the melted carbide is in contact with molten metal which is in a state of agitation. Instead of floating on the surface of the molten metal, 5 the carbide receptacle may be otherwise supported so that its outlet is in contact with the surface of the molten metal in the ladle or other container.

The required amount of carbide in lump form, 10 approximately 6 pounds per pound of sulphur to be removed, is placed in the receptacle. A flux such as sodium chloride may be added, if desired, to facilitate the reaction. The amount of flux, if any is employed, is not critical. The arc is 15 then started to melt the carbide. The molten carbide is mixed directly into the molten metal. The carbide reacts with sulphur in the molten metal, forming calcium sulphide which rises as a slag with the excess of calcium carbide and 20 may be removed. The sulphur content of the metal is thus reduced.

Referring to the drawing, 5 indicates an ingot mold or ladle of any suitable form and material which carries the bath of molten metal 6. Floating or otherwise supported on the bath 6 is a surrounding wall 7 of refractory material, not appreciably soluble in the metal bath, having a recess 8 affording a receptacle for the lumps of carbide 9. The receptacle has an opening 10 at its bottom which is submerged in the molten metal and beneath the surface thereof which is exposed to the atmosphere.

Electrodes 11 are arranged in suitable supports 12 so that their ends are contiguous. Conductors 13 are connected to the electrodes and to a source of current. While two electrodes are preferred, it is apparent that any other arrangement may be employed in accordance with well understood principles of electric furnace construction. Single electrode furnaces are well known in the art, as are submerged arc processes.

When a suitable amount of carbide has been placed in the receptacle surrounding the electrodes 11, the arc may be started. The resulting high temperature will melt the carbide, and the molten carbide in contact with the molten metal of the bath 6 will be disseminated therethrough as the result of agitation resulting from the operation of the arc. Thus all of the metal will be subjected to the desulphurizing activity of the calcium carbide and the sulphur thus removed will be separated in the slag which floats to the surface of the molten metal.

Various changes may be made in the form and construction of the apparatus and in the pro-

cedure as described without departing from the invention or sacrificing the advantages thereof.

The term "substantially pure calcium carbide" is used in the appended claims to define commercial carbide and to distinguish from slags which contain calcium carbide dissolved in or dispersed through other constituents of the slag.

I claim:

1. In the desulphurizing of molten iron and steel, the steps which comprise confining commercially pure calcium carbide to a relatively small restricted area on the surface of a body of the molten metal, melting the calcium carbide by means of an electric arc, thereby introducing the molten calcium carbide into the body of molten metal beneath the surface thereof while the molten metal is in a state of agitation to cause desulphurization of the metal.

2. In the desulphurizing of molten iron and 20

steel, the steps which comprise confining commercially pure calcium carbide to a relatively small restricted area on the surface of the molten metal, melting the calcium carbide by means of an electric arc, thereby causing the molten calcium carbide to diffuse into the molten metal and desulphurize the same.

3. In the desulphurizing of molten iron and steel, the steps which comprise confining commercially pure calcium carbide to a relatively small restricted area on the surface of the molten metal, melting the calcium carbide by an external source of heat, and introducing the molten carbide to the molten metal directly and beneath the surface thereof which is exposed to the atmosphere, whereby the molten calcium carbide is caused to diffuse into the molten metal and desulphurize the same.

JOHN J. CROWE.